

## UNITED STATES PATENT OFFICE

2,315,072

OXIDATION AND CORROSION INHIBITOR  
FOR LUBRICATING OILSJoseph F. Nelson and Raphael Rosen, Elizabeth,  
N. J., assignors to Standard Oil Development  
Company, a corporation of DelawareNo Drawing. Application July 26, 1939,  
Serial No. 286,566

20 Claims. (Cl. 252—48)

The present invention relates to improvements in types of blending agents characteristically containing constituents in a state which predisposes blends of these agents with lubricating oils to be corrosive to copper and similar metals. It is concerned particularly with rendering organic sulfide compounds, including polysulfide and hydroxyaryl sulfide anti-oxidants, non-corrosive to copper.

With developments in modern engines toward higher speeds and compression ratios, greater demands are made on lubricating oils for withstanding severe deteriorating conditions. Although well-refined mineral lubricating oils having desirable viscosity characteristics are suitably stable at low temperatures, when exposed to intense heat and oxidation at elevated temperatures in the operation of these modern high-speed engines, they tend to form sludge and varnish-like deposits. For this reason it is desirable to add to the oils substances which prevent such undesirable effects.

Furthermore with increased loads on power-drive mechanisms and increased adoption of such alloys as copper-lead cadmium-silver, or the like for construction of bearings used in these high-speed engines, critical demands are made also on the lubricants for film-forming qualities and for non-corrosiveness to such metals. For these reasons there has arisen the problem of imparting characteristics of improved oiliness and increased oxidation resistance to the oils. At the same time, the need for preventing corrosion of metal parts of the engines by lubricating compositions has become more acute.

Some definite improvements in the oxidation resistance of lubricating compositions have been made possible by the inclusion of compounds containing one or more non-metallic elements, belonging to the right-hand families of groups 5 and 6 of the periodic table, and which are chemically combined as in phenols, phenolic sulfides, thioamines, and similar types of compounds. In this connection, it has been found that anti-oxidants have higher effectiveness in stabilizing an oil and preventing corrosion of some metals, such as lead, when they contain sulfur, selenium, or tellurium in a state such that their blends in lubricants fail to pass a copper strip corrosion test.

In attempting to prevent copper strip corrosion by admixing corrosion inhibitors, more is lost than gained if the effectiveness of the sulfur family constituent for improving the oil composition is destroyed or substantially reduced.

With the object of eliminating corrosiveness of anti-oxidants to copper and similar metals, the present invention provides a method of chemically modifying such inhibitors by which enhancement of their oxidation inhibiting power and other desirable characteristics is also obtained.

The general method of improving an oxidation inhibiting compound having copper corroding tendencies is carried out in accordance with the present invention by treating the compound with a chemical modifying reactant, preferably in about stoichiometric or even less than stoichiometric proportion to the amount of corrosive component, at an elevated temperature, usually in the range of 100 to 300° C., which is below the temperatures at which either reactant undergoes thermal decomposition. This treatment is continued until the reactants are chemically combined or associated to yield an improved product, a blend of which in a lubricating oil will successfully pass a copper strip corrosion test. No part of the reaction product need be discarded, because the total reaction product serves as an excellent lubricating oil blending agent for inhibiting oxidation and corrosion during the period of service of the lubricating oil in a high-speed engine.

One type of modifying reactants found particularly effective is an ester of phosphorous acid, such as phenyl, benzyl, cresyl, or xylyl phosphites. Similarly, higher homologous aryl, alkaryl, or aralkyl phosphites may be used. An alkyl phosphite prepared from aliphatic alcohols, e. g., ethyl, propyl, butyl, or higher alcohols, may serve in the same capacity. The phosphite radicals also may be partly bound to metal constituents, as in salts. This type of modifying reactant, in removing the copper corroding tendencies from the oxidation inhibitors, leaves them remarkably well improved in color and in oxidation inhibiting action.

A second type of modifying reactants which may be used is a high boiling organic compound containing an unsaturated aliphatic group, which has at least 16 carbon atoms combined with hydrogen in a ratio ranging from about 15 to about 16.7 parts by weight of hydrogen per 100 parts by weight of carbon. For example, the tetramer of isobutene is an aliphatic compound with 16 carbon atoms, which has the maximum designated carbon to hydrogen ratio. Also, high molecular weight, unsaturated aliphatic acids or esters, olefin polymers, and petroleum components containing at least about 16 carbon atoms

per molecule and having a ratio of 15 to 16.7 parts by weight of hydrogen to 100 parts by weight of carbon are useful for the present purpose.

Among types of oxidation inhibitors which it is intended to modify in this manner are the phenolic and naphtholic compounds and, especially, their alkylated derivatives, including those which contain various substituents, such as amino groups, said compounds and their alkylated derivatives being preferably associated or combined with a sulfur family element. When sulfur, selenium, or tellurium constituents are absent from their molecules, these phenolic compounds are usually useful for inhibiting oxidation at only lower temperatures. Thus, alkylated phenols, e. g. cresols or higher alkyl phenols, naphthols, e. g. alpha or beta-naphthol, and di-hydroxy phenols, e. g. resorcinol, and similar substances are able to stabilize hydrocarbon oils at ordinary temperatures, but not very effectively at temperatures in the region above 200° C. Some metal salts of these compounds have greater effectiveness, e. g., phenolates of alkaline earth metals. By combining these compounds with sulfur so as to form their disulfides or polysulfides, their effectiveness for stabilizing oils against oxidation at the temperatures in excess of 200° C. which are encountered in modern engines is improved with attendant reduction of their corrosiveness to alloys such as copper-lead, etc.

In the high-temperature oxidation inhibitors, atoms of the sulfur family metalloid, that is, sulfur, selenium, or tellurium, may be attached directly to the rings of hydroxy aromatic radicals to form a linkage between said rings. It is preferred to have this linkage join 2 aryl groups containing hydroxyl and alkyl substituents, since such substituents give improved solubility and stability characteristics to the resulting compounds, but other compounds of this same general type may contain a substituted aromatic radical joined through a metalloid linkage to either a similar, substituted aromatic radical, an unsubstituted aromatic radical, or even an alkyl radical, as in the following formula.



wherein R represents an aromatic group which may contain one or more substituents of the class consisting of hydroxyl, amino, halogen, nitro, and alkyl radicals; R' is the same as R, or represents a group which is similar to R, or an aliphatic radical; and S, represents one or more atoms of a sulfur family metalloid. An excellent specific example of this type of oxidation inhibitor is the compound, di-tertiary-amyl-phenol disulfide, the structure of which may be represented as follows:



The substituents may be attached to the rings at other than the indicated positions. In general, these compounds are characterized by containing a metalloid having "corrosiveness" to copper as indicated by the copper strip test.

Other anti-oxidants have high-temperature, oxidation inhibiting properties and the characteristic of corrosiveness to copper of the compounds which have just been described. These include aromatic polysulfides, xanthates, thiocarbamates, thioxanthates, xanthogen, polysulfides, thiurams, etc. The following formulae illustrates some compounds of these types:



Still other substances useful as lubricating oil anti-oxidants include sulfurized plant and animal fatty oils and sulfurized hydrocarbon oils, which have had restricted application on account of their corrosiveness to copper.

In order to illustrate the method of improving these oxidation inhibiting compounds by rendering them non-corrosive to copper and the results therefrom, the following examples are presented.

**EXAMPLE 1**

A mixture of 15.6 g. of di-tertiary-amyl-phenol di-sulfide ( $C_5H_{11}\cdot C_6H_3\cdot OH\cdot$ )<sub>2</sub>-S<sub>2</sub>, which is black in appearance, and 14.1 g. of tri-cresyl phosphite (mixed in about a 1:1 mole ratio) was heated at 125 to 145° C. for 15 minutes, then, for an additional 15 minutes at 175 to 180° C., whereby a colorless, oily product was obtained.

Specific amounts of the resulting colorless product were added to portions of refined mineral lubricating oils and samples of these blends were tested to observe their action in corrosion tests and to evaluate the oxidation inhibiting properties of the modified di-sulfide inhibitor. Corrosion tests were made on an unblended mineral oil as a blank, on blends of the oil with the anti-oxidant before and after its modification, and on a blend of the oil with the unreacted modifying reactant. These tests were conducted under comparable conditions in the following manner and the results are presented in Table 1:

### COPPER STRIP CORROSION TEST

This consists in immersing a bright copper strip for 3 hours in the oil maintained at 212° F.; the presence of "corrosive" sulfur or of similar "corrosive" constituents in the oil is indicated by discoloration of the copper.

## LEAD TOLERANCE CORROSION TEST (OR UNDERWOOD TEST)

This test is used to determine the tendency of an oil to corrode bearings. 1500 cc. of the oil are maintained at 325° F. and are sprayed for 5 hours against two sets of bearings, one of copper-lead and the other of cadmium-silver alloy. The oil dripping from the bearings is recirculated. The bearings are weighed before and after the test to determine any loss in weight. The test is then repeated with addition of a soluble lead compound, preferably lead oleate, to the oil in increments of 0.005%, calculated on the basis of the weight of an equivalent amount of lead oxide. A loss in weight of 50 mg. or more in the cadmium-silver bearing indicates that the "lead tolerance" of the oil has been exceeded, and the amount of lead, computed as per cent lead oxide, added in the previous test is recorded

as the "lead tolerance." A lead tolerance of below 0.020% is considered unsatisfactory.

Table 1  
DATA ON CORROSION CHARACTERISTICS

| Lubricant composition                                                                                            | Percent inhibitor in the blend | Copper strip corrosion test | Lead tolerance percent PBO |
|------------------------------------------------------------------------------------------------------------------|--------------------------------|-----------------------------|----------------------------|
| Unblended oil (blank)                                                                                            | 0.00                           | Passed                      | 0.01                       |
| Unblended oil+di-tertiary-amyl-phenol disulfide (unmodified)                                                     | 0.125                          | Failed                      |                            |
|                                                                                                                  | .25                            | do                          | 0.075                      |
|                                                                                                                  | .50                            | do                          |                            |
|                                                                                                                  | 0.125                          | Passed                      |                            |
|                                                                                                                  | .25                            | do                          | 0.03                       |
|                                                                                                                  | .50                            | do                          |                            |
| Unblended oil+tricresyl phosphite                                                                                | 0.125                          | do                          |                            |
| Unblended oil+di-tertiary-amyl-phenol disulfide, modified by treatment with tricresyl phosphite as in Example 1. | 0.125                          | do                          | 0.06                       |
|                                                                                                                  | .25                            | do                          |                            |
|                                                                                                                  | .50                            | do                          |                            |

It is to be noted that the modified, sulfur-containing oxidation inhibitor successfully passes the copper strip corrosion test, thereby making its use more practical, whereas the unmodified, dark-colored compound fails to pass. Further, it is to be noted that when the tri-cresyl phosphite is employed alone as a blending agent, the oil blend barely passes the lead tolerance corrosion test, whereas the modified disulfide oxidation inhibitor is substantially as satisfactory as the unmodified disulfide inhibitor even though the disulfide ingredient forms only half the modified product, the other half comprising the tri-cresyl phosphite ingredient.

The relative value of an oxidation inhibitor, before and after its modification, for retarding oxidation of a lubricating oil at high temperatures is brought out in the following tests, the results of which are presented in Table 2.

Samples were prepared with a refined, light mineral lubricating oil, S. A. E. 20. Blank runs were made on the mineral oil containing no added oxidation inhibitor. Other test samples were blends of the same reference oil with 25% of the oxidation inhibitor before and after it was modified to eliminate its corrosiveness toward copper. These samples were subjected under comparable conditions to the following test:

#### OXIDATION RATE TEST

This consists in measuring the number of cc. of oxygen absorbed by 10 cc. of a lubricating composition sample during 15 minute periods at 200° C.

Table 2  
EVALUATION OF OXIDATION INHIBITING CHARACTERISTICS

| Lubricant composition                                                                                                 | Cc. oxygen absorbed in consecutive 15 minute periods per 10 cc. of oil |
|-----------------------------------------------------------------------------------------------------------------------|------------------------------------------------------------------------|
| Unblended oil (blank)                                                                                                 | 74-40-35                                                               |
| Unblended oil+0.25% di-tertiary-amyl-phenol disulfide (unmodified)                                                    | 34-20-21                                                               |
| Unblended oil+0.25% di-tertiary-amyl-phenol disulfide, modified by treatment with tricresyl phosphite as in Example 1 | 28-27-21                                                               |

These data demonstrate that the oxidation inhibiting properties of the modified oxidation inhibitor, which was treated to prevent its corrosion of copper and similar metals, are improved by this treatment. At the same time, the black colored inhibitor was converted into a colorless product, which is in itself a useful improvement.

Instead of modifying a high-temperature

oxidation inhibitor with only a phosphite to obtain desirable improvements of its corrosion inhibiting and oxidation inhibiting efficacies and color, as demonstrated, it may be modified with the second type of modifying reactant which enables it to reduce sludge formation in the oil, decreases its corrosiveness to copper, and also has beneficial effects on its oxidation inhibiting properties.

10 Sludge formation is particularly objectionable in lubricating oils subjected to the high temperatures encountered in high-speed engines because the sludge (oil-insoluble precipitate) tends to deposit on hot surfaces of valves, rings, and pistons, thereupon becoming carbonized to harmful hard coatings. The causes of sludge formation are not definitely known, even though sludge formation bears some relation to oxidation susceptibility of oils, for, rather anomalously, many oxidation inhibitors are notorious for increasing sludge formation in well-refined lubricating oils. Since phosphite modifying agents do not, as a general rule, improve anti-oxidants in this respect and have been observed to accentuate 15 sludging, it has been found desirable to remedy 20 this defect by modifying the anti-oxidants also by the reactants of the second type, which may be described as being sludge inhibiting modifiers.

The substances especially useful for reaction 25 with anti-oxidants to increase their sludge inhibiting tendencies as well as to reduce their tendencies toward corrosion of copper have, in general, the properties of high molecular weight polymers of iso-olefins, such as tetramers and higher polymers of isobutylene. Polymers of this 30 type are branched, open-chain hydrocarbons containing at least about 16 carbon atoms per molecule to which are attached hydrogen atoms in a ratio of at least 2 hydrogen atoms to each carbon atoms, as represented in the formula 35  $C_nH_{2n}$ . Other synthetic hydrocarbon oils obtainable by polymerization of cracked wax olefins also supply suitable modifying agents of this type. These substances may even be condensed with a relatively small quantity of cyclic hydrocarbons. The modifying agents should be free-flowing liquids, yet not readily volatile under ordinary conditions. Substances containing 40 more than 15 parts by weight of hydrogen to each 100 parts by weight of carbon and having 45 proper qualities to be used as this type of modifying reactant may be derived from petroleum oil fractions or naturally occurring fatty oils. Unsaturated, higher fatty acids, e. g. oleic acid, their esters and the like, which have hydrogen to carbon ratios above this lower limit may be used 50 in this connection. The heavier modifying reactants of this type are preferably used in smaller proportions than the lower molecular weight reactants.

55 The following examples illustrate the treatment of oxidation inhibitors with modifying agents which impart improved sludging properties as well as improved corrosion and oxidation inhibiting properties to the inhibitors.

#### EXAMPLE 2

One-tenth mole of di-tertiary-amyl-phenol disulfide was heated with 0.14 mole of tetra-isobutylene for 15 minutes at 230° to 235° C. and then for 20 minutes at 250° to 260° C. The resulting product, when blended with a refined mineral lubricating oil, was found to be non-corrosive in the copper strip test and improved for inhibiting sludge formation.

75 Using the same procedure with an unsaturated

oil, synthesized from cracked wax olefins by polymerization, in place of tetra-isobutylene, comparable results are achieved.

For testing sludging characteristics of the modified oxidation inhibitor, samples prepared by blending 0.2% of the modified inhibitor with a light lubricating oil, S. A. E. 20, were subjected to tests carried out in accordance with the procedure described in the Proc. A. S. T. M. 24, 964, II (1924) except for the time. This procedure consists in maintaining 10 g. of the sample in a flask with oxygen at atmospheric pressure at 200° C. for 24 hours, cooling the thus-treated oil, diluting it with naphtha, then separating the resulting precipitate by filtration after the mixture has stood for one hour at 25° C., and weighing the precipitate; the milligrams of precipitated sludge are known as the Sligh number. With each of the blends, a marked reduction of the Sligh number was observed as compared with that of the unblended oil.

Remarkable effects of the action of sludge inhibiting modifiers as a class on unblended oils can be illustrated by results obtained with oleic acid, which is a high molecular weight, unsaturated aliphatic compound containing at least 16 carbon atoms per molecule and having a ratio of 15.7 parts by weight of hydrogen to 100 parts by weight of carbon.

### EXAMPLE 3

Twenty-three g. of di-tertiary-amyl-phenol disulfide were treated with 17 g. of oleic acid,  $C_{17}H_{33}COOH$ , at 200° C. for 15 minutes. At the end of this period, a blend of the reaction product in a 1/2% concentration with a S. A. E. 20 refined mineral lubricating oil was found to pass the copper strip corrosion test. A blend of the unmodified disulfide reactant in only a 1/8% concentration with the same oil failed to pass this test. Portions of the modified reactant were tested in blends with a mineral lubricating oil for oxidation rate and sludging tendency. Using the same reference oil as described in Example 1, and conducting the tests under strictly comparable conditions, the following data were obtained:

Table 3

| Lubricant composition                                                                                          | Oxidation rate,<br>cc. $O_2$ (10 cc.<br>of oil) ab-<br>sorbed in 15<br>min. periods | Sligh<br>number,<br>mg. in<br>24 hrs. |
|----------------------------------------------------------------------------------------------------------------|-------------------------------------------------------------------------------------|---------------------------------------|
| Unblended oil (blank)                                                                                          | 74-40-35                                                                            | 4.9                                   |
| Unblended oil + 25% of di-tertiary-amyl-phenol disulfide modified by treatment with oleic acid as in example 3 | 16-22-12                                                                            | 1.2                                   |

Although the phosphite and the sludge inhibiting types of modifying reactants may be used separately, as illustrated in the examples which demonstrate their individual modifying effects, at times it may be more desirable to use a combination of the modifying reactants to obtain a maximum decrease in "corrosiveness" to copper and an increase in sludge inhibiting properties. For example, an anti-oxidant is rendered partially non-corrosive to copper by reaction with a phosphite, e. g. tri-phenyl phosphite, tri-cresyl phosphite, or the like, used in a proportion of about 1/4 or 1/2 mole to a mole of an anti-oxidant, such as a disulfide, and is fully modified by further reaction with a fraction of a mole of a sludge inhibiting modifier, e. g. the olefin polymers, unsaturated fatty acid compounds, and the like.

The order in which each type of modifying reactant is used in the treatment is not of great importance, but it is preferred to limit the proportions of modifying reactants to avoid excessive diminution in the concentration of the anti-oxidant. In some instances, it may be preferred to use the sludge inhibiting modifier first to improve the anti-oxidant to some extent, and then to complete the treatment with phosphite.

With anti-oxidants containing no more than 2 sulfur family constituents per molecule, e. g., disulfides, monosulfides, or monoselenides, etc., the modifying reactants singly or combined are used preferably in proportions ranging from about 1/2 mole to 1 1/2 moles for each mole of the anti-oxidant compound. In polysulfides, which have a higher content of sulfur, larger proportions of modifying reactants are required. For a mixture of a disulfide with a monosulfide, or for a monosulfide alone, wherein "corrosiveness" to copper may be due mainly to the presence of free sulfur as an impurity, less than 1 mole of modifying reactant need be used for each mole of the substance to be modified.

In any event, the phosphite performs the function of improving color and unsaturated aliphatic reactants serve to improve sludging characteristics, while both types of reactants contribute to removal of the "corrosiveness" to copper and improvement of oxidation inhibiting power of the anti-oxidants.

As previously noted, the reaction products result from the union of the modifying reactants with the anti-oxidants without splitting off any components or constituents. The reaction may be looked upon as an addition reaction, although some rearrangement may occur. In this respect, the reaction is different from a condensation reaction, which involves the separation of constituents and in which the procedure is frequently complicated by the presence of catalysts and the formation of undesirable sludges.

For increasing the stability of lubricating oils, the modified anti-oxidants of this invention are generally to be blended therein in concentrations ranging from about .1 to about 2% by weight. In some instances, higher concentrations may be preferred, e. g., 5% or more. The improved blending agents are effective in many types of petroleum products irrespective of source or method of refining. The colorless product is particularly valuable for use in white oils procured generally by refining paraffinic, naphthenic, or mixed crude oil fractions of these types to a high degree by treatments involving the use of strong mineral acids, e. g., concentrated or fuming sulfuric acid, clay, solvent extraction, hydrogenation, aluminum chloride-type compounds, or other reagents and procedures. Selection of the particular mode of modifying the anti-oxidant may be based on the particular use of the product. For some purposes, the anti-oxidant is preferably modified to avoid sludging. Also, the modified anti-oxidants may be intermixed or used together with other compounds having known oxidation inhibiting action.

While the present invention is mainly directed to improved blending agents for motor oils, it is not limited entirely to this field because these agents are useful in insulating oils, in high pressure lubricants for gears, industrial oils, greases, etc. They may be used in many types of mineral oils which perform lubricating functions, including those employed in Diesel engines, and may be used with admixtures of fatty oils, soaps

of fatty acids or phenols, pour point depressants, viscosity improving agents, and other agents used for improving lubricants.

This invention is not to be limited by any theory of reaction or inhibiting activity. The description and examples are illustrative only and any modification or variation therefrom which conforms to the spirit of the invention is intended to be included within the scope of the claims.

We claim:

1. Process of improving a high-temperature oxidation inhibitor containing a sulfur family element in a state corrosive to copper and similar metals, which consists in reacting said oxidation inhibitor with modifying reactants comprising a phosphite and an unsaturated aliphatic type compound containing at least 16 carbon atoms per molecule with a ratio of about 15 to 16.7 parts by weight of hydrogen to each 100 parts by weight of carbon, and heating the mixture to an elevated temperature for a sufficient period of time to form a lubricating oil blending agent which avoids corrosion of copper.

2. A process as described in claim 1 in which said oxidation inhibitor reacted with said modifying reactant is an organic polysulfide.

3. Process of improving a lubricating oil anti-oxidant of the type containing a corrosive sulfur family metalloid which comprises mixing the anti-oxidant with an unsaturated aliphatic compound having at least about 16 carbon atoms per molecule and a ratio of about 15 to 16.7 parts by weight of hydrogen to each 100 parts by weight of carbon, and heating the mixture at an elevated temperature for a period sufficient to decrease the copper corrosion tendency of the anti-oxidant when blended in a refined mineral lubricating oil.

4. A process in accordance with claim 3, in which said unsaturated aliphatic compound is a polymer of an iso-olefin hydrocarbon.

5. A process in accordance with claim 3, in which said unsaturated aliphatic compound is a carboxylic compound.

6. A process of modifying a lubricating oil anti-oxidant of the type containing a corrosive sulfur family metalloid which comprises reacting the anti-oxidant at an elevated temperature in admixture with an unsaturated aliphatic compound having at least about 16 carbon atoms combined with hydrogen in a ratio of about 15 to 16.7 parts by weight of hydrogen to each 100 parts by weight of carbon for a period sufficient to at least partially reduce copper corrosion tendencies of the anti-oxidant, then further heating the resulting product with an admixed phosphite at an elevated temperature to render the product completely non-corrosive to copper.

7. A process for the production of an improved oxidation inhibitor from a hydroxy aryl compound containing a combined metalloid selected from the class consisting of sulfur, selenium, and tellurium, which comprises heating the hydroxy aryl compound to an elevated temperature in the range of about 100° C. to about 300° C. with an admixed organic compound containing an unsaturated aliphatic group and having at least 16 carbon atoms combined with hydrogen in a ratio of 15 to 16.7 parts by weight of hydrogen to each 100 parts by weight of carbon, and maintaining the hydroxy aryl compound at the elevated temperature with a sufficient proportion of said organic compound for a period sufficient to decrease sludging and copper corrosion tendencies

when said product is used as an inhibitor in a refined mineral lubricating oil.

8. An improved anti-oxidant composition consisting essentially of an anti-oxidant, containing sulfur corrosive to copper, chemically combined in an addition product with a compound containing a phosphite radical and an organic compound containing an unsaturated aliphatic group and having at least 16 carbon atoms combined with hydrogen in a ratio of 15 to 16.7 parts by weight of hydrogen to each 100 parts by weight of carbon, said composition being non-corrosive to copper when used as an inhibitor in a refined lubricating oil.

10 15 20 25 30 35 40 45 50 55 60 65 70 75

9. An improved anti-oxidant composition consisting essentially of an organic sulfide combined in an addition product with a phosphite ester, said addition product being characterized by being substantially colorless and by being non-corrosive to copper when used as an inhibitor in a refined mineral lubricating oil.

10. An improved anti-oxidant composition consisting essentially of an organic sulfide combined in an addition product with an unsaturated aliphatic compound having at least 16 carbon atoms combined with hydrogen in a ratio of 15 to 16.7 parts by hydrogen to each 100 parts by weight of carbon, said addition product being non-corrosive to copper and decreasing sludging tendencies when used as an inhibitor in a refined mineral lubricating oil.

11. An improved anti-oxidant composition consisting essentially of a hydroxy aryl disulfide combined in an addition product with a phosphite ester, said addition product being characterized by being substantially colorless and by being non-corrosive to copper when used as an inhibitor in a refined mineral lubricating oil.

12. An improved anti-oxidant composition consisting essentially of a hydroxy aryl disulfide combined in an addition product with an organic compound containing an unsaturated aliphatic group and having at least 16 carbon atoms combined with hydrogen in a ratio of 15 to 16.7 parts by weight of hydrogen to each 100 parts by weight of carbon, said addition product being characterized by being non-corrosive to copper and by causing decreased sludging tendencies of the oil when used as an inhibitor in a refined mineral lubricating oil.

13. A composition comprising an oil-soluble chemical reaction product of a hydroxy aryl disulfide and a material selected from the group consisting of at least partially organic esters of phosphorous acid and high-boiling organic compounds containing an unsaturated aliphatic group and having at least 16 carbon atoms combined with hydrogen in a ratio of about 15 to 16.7 parts by weight of hydrogen to each 100 parts by weight of carbon, said reaction product being non-corrosive to copper.

14. A composition comprising an oil-soluble chemical reaction product of a sulfide of an alkylated phenolic compound, and an unsaturated aliphatic compound having at least 16 carbon atoms and containing at least 15 parts by weight of hydrogen to each 100 parts by weight of carbon.

15. A lubricating composition comprising a major proportion of a mineral lubricating oil base stock into which has been incorporated a small amount of a preformed chemical reaction product of an organic sulfur compound and unsaturated aliphatic compounds having at least 16 carbon atoms and containing at least 15 parts by

weight of hydrogen to each 100 parts by weight of carbon, said lubricant being substantially non-corrosive to copper.

16. A lubricating composition non-corrosive to copper, comprising a major proportion of mineral lubricating oil base stock into which has been incorporated a small amount of a preformed chemical reaction product of a dialkyl phenol disulfide and an organic phosphite.

17. A lubricating composition non-corrosive to copper, comprising a major proportion of mineral lubricating oil base stock into which has been incorporated a small amount of a preformed chemical reaction product of a metal salt of an alkyl phenol sulfide and a substance selected from the group consisting of organic phosphites and unsaturated aliphatic compounds having at least 16 carbon atoms and containing at least 15 parts by weight of hydrogen to each 100 parts by weight of carbon.

18. The method of lubricating bearings containing a metal such as copper, cadmium, silver, and lead, having substantial susceptibility to corrosion by sulfur compounds, which consists in applying to said bearing surfaces a lubricant comprising a major proportion of mineral lubricating oil base stock into which has been incorporated a small amount of a preformed chemical reaction product of a hydroxyl aryl disulfide having oxidation-inhibiting properties but normally corrosive to copper, with an organic phosphite,

said lubricant being non-corrosive to said bearings.

19. A lubricating composition comprising a major proportion of mineral lubricating oil base stock into which has been incorporated not substantially more than 0.25% of a reaction product of a hydroxy aryl disulfide and a material selected from the group consisting of at least partially organic esters of phosphorous acid and high-boiling organic compounds containing an unsaturated aliphatic group and having at least 16 carbon atoms combined with hydrogen in a ratio of about 15 to 16.7 parts by weight of hydrogen to each 100 parts by weight of carbon, said reaction product being non-corrosive to copper.

20. A substantially colorless mineral oil composition comprising a major proportion of a mineral white oil, not more than about 0.25% by weight of a substantially colorless to clear light colored reaction product of a hydroxy aryl disulfide and a material selected from the group consisting of at least partially organic esters of phosphorous acid and high-boiling organic compounds containing an unsaturated aliphatic group, and having at least 16 carbon atoms combined with hydrogen in a ratio of about 15 to 16.7 parts by weight of hydrogen to each 100 parts by weight of carbon, said reaction product being non-corrosive to copper.

JOSEPH F. NELSON.  
RAPHAEL ROSEN.